

# United States Patent

[19]

Yanai

[11] 3,854,869

[45] Dec. 17, 1974

[54] **METHOD OF IMPARTING CREASE  
RESISTANCE TO CELLULOSIC FIBERS BY  
TREATING THEM WITH  
TETRAOXYMETHYLENE**

[75] Inventor: **Yuichi Yanai**, Okazaki, Japan

[73] Assignee: **Nisshin Boseki Kabushiki Kaisha**,  
Tokyo, Japan

[22] Filed: **Aug. 10, 1972**

[21] Appl. No.: **279,362**

[52] U.S. Cl. .... **8/116.4, 8/116 R**

[51] Int. Cl. .... **D06m 13/12, D06m 13/14**

[58] Field of Search ..... **8/116 R, 116.4**

[56] **References Cited**

UNITED STATES PATENTS

|           |        |                 |       |         |
|-----------|--------|-----------------|-------|---------|
| 3,165,374 | 1/1965 | Husebeck et al. | ..... | 8/116.4 |
| 3,173,751 | 3/1965 | Daul et al.     | ..... | 8/116.4 |

|           |        |                    |         |
|-----------|--------|--------------------|---------|
| 3,676,053 | 7/1972 | Miyake et al. .... | 8/116.4 |
| 3,679,348 | 7/1972 | Asahi et al. ....  | 8/116.4 |

**OTHER PUBLICATIONS**

Pierce et al., American Dyestuff Reporter, May, 1970,  
p. 50.

Reid et al., Textile Chemist and Colorist, 3, (8),  
51-53, (1971).

*Primary Examiner*—George F. Lesmes

*Assistant Examiner*—J. Cannon

*Attorney, Agent, or Firm*—Robert E. Burns;  
Emmanuel J. Lobato; Bruce L. Adams

[57] **ABSTRACT**

This invention is to provide a method of imparting  
crease resistance and soft touch to cellulosic fibers or  
textile fabrics and knitted goods containing cellulosic  
fibers by treating them with tetraoxymethylene in the  
presence of a certain catalytic mixture.

**4 Claims, No Drawings**

**METHOD OF IMPARTING CREASE RESISTANCE  
TO CELLULOSIC FIBERS BY TREATING THEM  
WITH TETRAOXYMETHYLENE**

**DETAILED EXPLANATION OF THE INVENTION**

This invention relates to a method of imparting crease resistance and soft touch to cellulosic fibers or textile fabrics and knitted goods containing cellulosic fibers by treating them with tetraoxymethylene in the presence of a catalytic mixture of a certain metalboron fluoride and a certain organic carboxylic acid.

It is known that tetraoxymethylene is a cyclic tetramer of formaldehyde ( $\text{CH}_2\text{O}$ ) and that it is a needle-like crystal which has the melting point of 112°C and is difficult in liberating free formaldehyde in comparison with other derivatives of formaldehyde. Tetraoxymethylene has been reported by Staudinger and et al. in *Helv. Chim. Acta* 848, 65 published in the year 1925 but it has not yet been used in the industrial field until today because an industrial and economical method for the production of tetraoxymethylene has not been developed.

Now, some industrial and economical methods for the production of tetraoxymethylene are proposed and they are explained in Japanese Patent Publication Nos. 5352/69, 2222/69, 16751/68 and 28460/68, and as a result, the industrial way for utilizing tetraoxymethylene has been opened.

Also, Japanese Patent Publication Nos. 21356/65, 8877/66, 953/67 and 23635/68 disclose methods for utilizing tetraoxymethylene and it is noted that they relate to the use of tetraoxymethylene as a raw material for the production of high molecular materials but they do not relate to the use of tetraoxymethylene for treating cellulosic fibers. Further, U.S. Pat. No. 3,186,945 discloses the use of a catalyst comprising an organic acid such as citric acid and a metal salt of Lewis type acid for thermally treating free aldehydes or some compounds capable of liberating free aldehydes or thermally reactive aldehyde resins. It is noted in claims and Examples of the U.S. Patent that formaldehyde or methylol triazone is used in the presence of a catalyst comprising citric acid and hexahydrated magnesium nitrate in the weight ratio of 2:7, which is referred as to a 2-7 catalyst or a catalyst comprising citric acid, strontium nitrate and hexahydrated magnesium nitrate in the weight ratios of 2:3:4, which is referred as to a 2-3-4 catalyst or a catalyst comprising citric acid and hexahydrated magnesium nitrate in the weight ratio of 5:12, which is referred as to a 5-12 catalyst, but it is noted that the U.S. Patent does not disclose the use of tetraoxymethylene and a catalytic mixture of a metalboron fluoride and an organic carboxylic acid used in accordance with this invention. It was found that the 2-7 catalyst, 2-3-4 catalyst and 5-12 catalyst vary greatly in their effects depending on the temperature and are less effective as the catalysts for tetraoxymethylene and so they can not be used practically when cellulosic fibers or textile fabrics and knitted goods containing the cellulosic fibers are treated with tetraoxymethylene.

Still further, the American Dyestuff Reporter, Vol. 57 (1968), page 864 discloses the use of an active catalyst comprising a metal halide and a hydroxy — or an alkoxy — substituted carboxylic acid but it is noted that the active catalyst is different from the catalytic mix-

ture of metal-boron fluoride and an organic carboxylic acid used in accordance with this invention. Also it was found that such an active catalyst can not be used as a catalyst for tetraoxymethylene.

The inventor has investigated various methods for a long time in which tetraoxymethylene is used for imparting crease resistance to cellulosic fibers or textile fabrics and knitted goods containing cellulosic fibers and as a result, the inventor has discovered this invention in which tetraoxymethylene can be practically used in the presence of a catalytic mixture of at least one of metal-boron fluorides and at least one of organic carboxylic acids as listed below.

Namely, some examples of the metal-boron fluorides are magnesium-boron fluoride, aluminum-boron fluoride, zinc-boron fluoride, cadmium-boron fluoride, tin-boron fluoride and lead-boron fluoride. Also some examples of the organic carboxylic acids are formic acid, oxalic acid, malonic acid, succinic acid, maleic acid, maleic acid anhydride, glycollic acid, lactic acid, malic acid, citric acid and tartaric acid. It is preferable to use the water soluble metal-boron fluorides and organic carboxylic acid.

The advantageous merits achieved in accordance with this invention by using tetraoxymethylene for imparting crease resistance to cellulosic fibers or textile fabrics and knitted goods containing cellulosic fibers are summarized as follows.

1. An excellent soft touch is imparted to the finished products contrary to the amino-plastic resins which impart rough touch to the finished products. It is considered that such a merit is achieved on the basis of the facts that tetraoxymethylene can easily be penetrated into the cellulosic fibers and also that the self-polymerization of tetraoxymethylene and the formation of the resinous products are prevented on the surfaces of the cellulosic fibers as tetraoxymethylene is sublimated at elevated temperatures.

2. Tetraoxymethylene is the tetramer of formaldehyde not containing a nitrogen atom or atoms contrary to the resinous substances, which are used as the usual anti-creasing agents, containing a nitrogen atom or atoms and therefore the cellulosic fibers or the textile fabrics and knitted goods containing the cellulosic fibers are not degraded in their quality due to the absorption of chlorine but they are improved in their light-resistance and thermal resistance.

3. The chemicals required for treating textile fabrics and knitted goods are reduced in amount to about 30% of the glyoxal-monourea type resins in order to impart the same degree of crease resistance to such textile fabrics.

4. Formaldehyde is retained in a very small amount or not retained in the finished textile fabrics and knitted goods and so they can be used freely due to absence of bad effects on the health.

Now, in the art there is an important problem in that mechanical strength of the finished textile fabrics is remarkably reduced when tetraoxymethylene is used in the presence of the known catalysts which are used in combination with the usual anti-creasing agents and therefore, in such a case, it is necessary to control exactly the conditions for treating the textile fabrics in order to keep their mechanical strength at the degree required for the practical use and simultaneously to achieve the crease resistance required for practical use.

As it is obvious from the description indicated hereinafter, the crease resistance and mechanical strength of the finished textile fabrics are distinguishably varied depending on the heating temperature when the known catalysts are used and therefore it is impossible to control the conditions for treating the textile fabrics for producing the finished stable and crease-resistance products. Also, the known catalysts have a weak catalytic effect on tetraoxymethylene and therefore it is necessary to use tetraoxymethylene at elevated temperatures in order to impart satisfactory crease resistance to cellulosic fibers or the textile fabrics and knitted goods containing the cellulose fibers; it was found in such a case that the textile fabrics become brittle and are yellow colored and so the finished products are of no practical use.

On the contrary, the catalytic mixture used in this invention can be used in the wide ranges of heating temperatures used to impart the crease resistance to the textile fabrics, and the resultant textile fabrics have neither decreased mechanical strength nor were they yellow colored. Therefore, the catalytic mixture of this invention is the most important to achieve crease resistance of the cellulosic fibers when they are treated with tetraoxymethylene and it can be said that it is a new discovery by the inventor to use tetraoxymethylene for imparting crease resistance to cellulosic fibers.

It is preferable to use the metal-boron fluorides in an amount of 0.02 to 10.0% by weight of the textile fabrics and knitted goods containing the cellulosic fibers and also it is preferable to use the organic carboxylic acids in an amount of 0.02 to 10.0% by weight of the textile fabrics and knitted goods. It is noted that the cellulosic fibers and textile fabrics can be treated for a short period of time at a lower temperature as the amount of the catalytic mixture increases. In such a case, the cellulosic fibers tend to decompose and therefore the concentration of the catalytic mixture used in this invention must be adjusted depending on the conditions of the heat treatment for the cellulosic fibers.

Tetraoxymethylene can be used in an amount of 0.1 to 10.0% by weight of the cellulosic fibers or the textile fabrics and knitted goods and it is preferable to use tetraoxymethylene in an amount of 0.3 to 4.0% by weight of the cellulosic fibers or the textile fabrics.

Tetraoxymethylene can be applied onto the cellulosic fibers or the textile fabrics by dipping them into

sprayed cellulosic fibers or textile fabrics in the same manner as in the prior known techniques.

It is an easy procedure to use a single solution in which tetraoxymethylene and the catalytic mixture are dissolved but it is possible to use them in a separate step. Some examples of solvents used for dissolving tetraoxymethylene are organic solvents such as acetone, nitromethane and halogenated hydrocarbons but it is preferable in practice to use water as the solvent.

The cellulosic fibers or the textile fabrics and knitted goods containing the cellulosic fibers thus treated with tetraoxymethylene and the catalytic mixture of this invention are dried and then subjected to a heat treatment. It is necessary to take care in handling the dried materials because tetraoxymethylene is sublimated when the dried materials are left for some time as they are.

The heat treatment can be carried out at a temperature of 100°C to 220°C and it is preferable to carry out the heat treatment at a temperature of 120°C to 180°C for 1 to 3 minutes. It is noted that the time required for the heat treatment can be shortened as the heating temperature increases. Also it is noted that the heat treatment can be conducted by using a hot air, a heated oil, a molten metal bath, a heated roll, a hot press and other devices.

It is obvious to those skilled in the art that tetraoxymethylene and the catalytic mixture used in accordance with this invention can be used in combination with various kinds of assistants such as softeners, finishing agents, soil-release agents, water-proofing agents, antistatic agents and flame-proofing agents for imparting a desirable quality to the finished textile fabrics and knitted goods.

This invention is illustrated by the following Examples.

#### EXAMPLE 1

40 Each of eight test samples of scoured, bleached and mercerized cotton cloth, which is woven of the warps of 40 yarn counts and the wefts of 30 yarn counts, and has the weight of 125 grams/square meter, was dipped into each of aqueous solutions 1 to 8 which are prepared by mixing water (as a solvent) and the chemical agents as indicated in the following Table 1 in the indicated grams per 100 cc of the aqueous solution.

Table 1

| Chemical Agents                 | Nos. of Aqueous Solutions |     |     |     |     |     |     |     |
|---------------------------------|---------------------------|-----|-----|-----|-----|-----|-----|-----|
|                                 | 1                         | 2   | 3   | 4   | 5   | 6   | 7   | 8   |
| Zinc-boron fluoride (45%)       | 1.5                       | 2.0 |     |     |     |     |     |     |
| Hexahydrated zinc nitrate       |                           |     | 3.0 |     |     |     |     |     |
| Hexahydrated magnesium chloride |                           |     |     | 2.0 |     |     |     |     |
| Hexahydrated magnesium nitrate  |                           |     |     |     | 1.4 | 0.8 | 1.5 | 1.0 |
| Anhydrous strontium nitrate     |                           |     |     |     |     | 0.6 |     |     |
| Monohydrated citric acid        | 0.5                       |     |     |     | 0.4 | 0.4 | 0.6 | 0.5 |
| Tetraoxymethylene               | 3.0                       | 3.0 | 3.0 | 3.0 | 3.0 | 3.0 | 3.0 | 3.0 |
| Polyethylene softener           | 2.0                       | 2.0 | 2.0 | 2.0 | 2.0 | 2.0 | 2.0 | 2.0 |

Note:

- (1) Aqueous solution No. 1 was prepared by using the catalytic mixture of this invention.
- (2) Aqueous solution No. 5 was prepared by using the 2-7 catalyst disclosed in the U.S. Pat. 3,186,954.
- (3) Aqueous solution No. 6 was prepared by using the 2-3-4 catalyst disclosed in the U.S. Pat. 3,186,954.
- (4) Aqueous solution No. 7 was prepared by using the 5-12 catalyst disclosed in the U.S. Pat. 3,186,954.
- (5) Aqueous solution No. 8 was prepared by using the active catalyst disclosed in the American Dyestuff Reporter, Vol. 57 (1968), page 864.

a tetraoxymethylene-containing solution or by spraying the tetraoxymethylene-containing solution on to them and then by squeezing or dehydrating the dipped or

Then the dipped test samples were mangled to a wet pick-up of about 70% and dried in a non-touched drier at 125°C for 90 seconds and then the dried test samples

were heat-treated in a pilot baking machine at 130°C for 2 minutes or 140°C for 2 minutes or 160°C for 2 minutes and then the heat-treated test samples were washed with a neutral soap solution and dried in a tumbler type drier. The dried test samples were tested for the degree of crease resistance by using the test method disclosed in AATCC, 661968 and also they were tested for tear strength by using the pendulum method disclosed in the Japanese Industrial Standards L 1004-1959. The test results are given in the following Table 2.

5

useful for treating the cotton cloth with tetraoxymethylene but also that other catalysts are not suitable.

#### EXAMPLE 2

Eight test samples were prepared by using a cloth which is woven of a mixed yarn having the 40 counts and consisting of polyester fibers (65%) and cotton fibers (45%). The test samples were scoured, bleached, mercerized and heat-set. Each of the test samples was dipped into each of the aqueous solutions 1 to 8 dis-

10

Table 2

| Nos. of Test samples | Nos. of Aqueous solutions | Heat-treated at (°C) | Crease Recovery Angle (dry) | Tear Strength(g) in the direction of the warp |
|----------------------|---------------------------|----------------------|-----------------------------|-----------------------------------------------|
| 1                    | 1                         | 130                  | 278                         | 523                                           |
|                      |                           | 140                  | 280                         | 510                                           |
|                      |                           | 160                  | 282                         | 505                                           |
| 2                    | 2                         | 130                  | 228                         | 740                                           |
|                      |                           | 140                  | 254                         | 532                                           |
|                      |                           | 160                  | 277                         | 438                                           |
| 3                    | 3                         | 130                  | 190                         | 1038                                          |
|                      |                           | 140                  | 200                         | 955                                           |
|                      |                           | 160                  | 239                         | 725                                           |
| 4                    | 4                         | 130                  | 237                         | 583                                           |
|                      |                           | 140                  | 251                         | 433                                           |
|                      |                           | 160                  | 266                         | 375                                           |
| 5                    | 5                         | 130                  | 221                         | 768                                           |
|                      |                           | 140                  | 254                         | 665                                           |
|                      |                           | 160                  | 294                         | 495                                           |
| 6                    | 6                         | 130                  | 210                         | 950                                           |
|                      |                           | 140                  | 254                         | 770                                           |
|                      |                           | 160                  | 273                         | 425                                           |
| 7                    | 7                         | 130                  | 235                         | 707                                           |
|                      |                           | 140                  | 257                         | 572                                           |
|                      |                           | 160                  | 287                         | 432                                           |
| 8                    | 8                         | 130                  | 248                         | 537                                           |
|                      |                           | 140                  | 273                         | 452                                           |
|                      |                           | 160                  | 293                         | 338                                           |

As it is obvious from the Table 2, the test sample 1 is not changed in its crease resistance and tear strength even if it is heat-treated at 130°C or 140°C or 160°C but the test samples 2 to 8 are widely changed in their crease resistance and tear strength after they are heat-treated at the different heating temperature. This proves that the catalytic mixture of this invention is

closed in Example 1 and then they were heat-treated in the same manner as in Example 1. The resultant test samples were tested for their wash and wear rating by using the I-B method disclosed in AATCC, 124-1967 and also they were tested for tear strength in the same manner as in Example 1. The test results are given in the following Table 3.

Table 3

| Nos. of Test samples | Nos. of Aqueous solutions | Heat-treated at (°C) | Wash and Wear Rating (Grade) | Tear Strength(g) in the direction of the weft |
|----------------------|---------------------------|----------------------|------------------------------|-----------------------------------------------|
| 1                    | 1                         | 130                  | 3.8                          | 1345                                          |
|                      |                           | 140                  | 3.8                          | 1320                                          |
|                      |                           | 160                  | 3.8                          | 1333                                          |
| 2                    | 2                         | 130                  | 3.0                          | 1406                                          |
|                      |                           | 140                  | 3.2                          | 1370                                          |
|                      |                           | 160                  | 3.5                          | 1286                                          |
| 3                    | 3                         | 130                  | 2.5                          | 1413                                          |
|                      |                           | 140                  | 2.7                          | 1430                                          |
|                      |                           | 160                  | 3.1                          | 1272                                          |
| 4                    | 4                         | 130                  | 3.0                          | 1385                                          |
|                      |                           | 140                  | 3.2                          | 1370                                          |
|                      |                           | 160                  | 3.3                          | 1242                                          |
| 5                    | 5                         | 130                  | 2.8                          | 1382                                          |
|                      |                           | 140                  | 3.3                          | 1313                                          |
|                      |                           | 160                  | 4.2                          | 1120                                          |
| 6                    | 6                         | 130                  | 2.7                          | 1357                                          |
|                      |                           | 140                  | 3.2                          | 1334                                          |
|                      |                           | 160                  | 3.5                          | 1218                                          |
| 7                    | 7                         | 130                  | 3.1                          | 1403                                          |
|                      |                           | 140                  | 3.3                          | 1324                                          |
|                      |                           | 160                  | 3.7                          | 1261                                          |
| 8                    | 8                         | 130                  | 3.2                          | 1378                                          |
|                      |                           | 140                  | 3.5                          | 1290                                          |
|                      |                           | 160                  | 4.0                          | 1194                                          |

As it is obvious from the Table 3, the test sample 1 has the good and stable wash and wear rating but other samples 2 to 8 are changed in their wash and wear rating depending on the variation of heating temperature. This proves that the catalytic mixture of this invention is practically useful but the other known catalysts are not suitable for treating the textile fabric containing cellulosic fibers.

## EXAMPLE 3

Example 1 was repeated with the exception that

are practically useful for treating the textile fabric containing cellulosic fibers.

## EXAMPLE 4

Example 1 was repeated with the exception that aqueous solutions 18 to 22 were used. The aqueous solutions 18 to 22 were prepared by mixing water (as a solvent) and the chemical agents as indicated in the following Table 5 in the indicated grams per 100 cc of the aqueous solution.

Table 5

| Chemical Agents               | Nos. of Aqueous Solutions |     |     |     |     |
|-------------------------------|---------------------------|-----|-----|-----|-----|
|                               | 18                        | 19  | 20  | 21  | 22  |
| Magnesium-boron fluoride(40%) | 1.4                       |     |     |     |     |
| Aluminum-boron fluoride(30%)  |                           | 1.4 |     |     |     |
| Cadmium-boron fluoride(50%)   |                           |     | 3.0 |     |     |
| Tin-boron fluoride(47%)       |                           |     |     | 1.4 |     |
| Lead-boron fluoride(50%)      |                           |     |     |     | 2.5 |
| Monohydrated citric acid      | 0.5                       | 0.5 | 0.5 | 0.5 | 0.5 |
| Tetraoxymethylene             | 3.0                       | 3.0 | 3.0 | 3.0 | 3.0 |
| Polyethylene(softener)        | 2.0                       | 2.0 | 2.0 | 2.0 | 2.0 |

aqueous solutions 9 to 17 were used. The aqueous solutions 9 to 17 were prepared by mixing 3.0 grams/100 cc of tetraoxymethylene, 2.0 grams/100 cc of polyethylene softener and 1.5 grams of a 45% solution of zinc-boron fluoride/100 cc with 0.5 gram/100 cc of an organic carboxylic acid selected from the group consist-

30

The resultant test samples 18 to 22 were tested their crease resistance and tear strength in the same manner as in Example 1. The test results are given in the following Table 6. As it is obvious from the Table 6, the test samples 18 to 22 have the good and stable crease resistance and tear strength. Also it was found that all the

Table 6

| Nos. of Test Samples | Nos. of Aqueous Solutions | Crease Recovery Angle(dry) |       |       | Tear Strength(g) in the direction of the warp |       |       |
|----------------------|---------------------------|----------------------------|-------|-------|-----------------------------------------------|-------|-------|
|                      |                           | 130°C                      | 140°C | 160°C | 130°C                                         | 140°C | 160°C |
| 18                   | 18                        | 282                        | 280   | 287   | 480                                           | 463   | 418   |
| 19                   | 19                        | 261                        | 267   | 278   | 573                                           | 540   | 527   |
| 20                   | 20                        | 251                        | 254   | 260   | 580                                           | 543   | 540   |
| 21                   | 21                        | 252                        | 256   | 271   | 478                                           | 500   | 447   |
| 22                   | 22                        | 260                        | 259   | 266   | 537                                           | 520   | 497   |

ing of (9) formic acid, (10) dihydrated oxalic acid, (11) malonic acid, (12) succinic acid, (13) maleic acid, (14) glycollic acid, (15) lactic acid, (16) malic acid and (17) tartaric acid. The resultant test samples 9 to 17 were tested for their crease resistance and tear strength in the same manner as in Example 1. The test results are given in the following Table 4. As it is obvious from the Table 4, the test samples 9 to 17 have the good and stable crease resistance and tear strength. This proves that the catalytic mixtures of this invention

45 test samples are soft touch and improved in their thermal resistance, light-resistance and chlorine-resistance.

## EXAMPLE 5

Example 1 was repeated with the exception that aqueous solutions 23 to 28 were used. The aqueous solutions 23 to 28 were prepared by mixing water (as a solvent) and the chemical agents as indicated in the following Table 7 in the indicated grams per 100 cc of the aqueous solution.

Table 4

| Nos. of Test Samples | Nos. of Aqueous Solutions | Crease Recovery Angle(dry) |       |       | Tear Strength (g) in the direction of the warp |       |       |
|----------------------|---------------------------|----------------------------|-------|-------|------------------------------------------------|-------|-------|
|                      |                           | 130°C                      | 140°C | 160°C | 130°C                                          | 140°C | 160°C |
| 9                    | 9                         | 278                        | 280   | 181   | 525                                            | 517   | 457   |
| 10                   | 10                        | 282                        | 285   | 286   | 310                                            | 325   | 318   |
| 11                   | 11                        | 278                        | 280   | 284   | 438                                            | 418   | 480   |
| 12                   | 12                        | 274                        | 277   | 282   | 482                                            | 455   | 422   |
| 13                   | 13                        | 254                        | 257   | 259   | 520                                            | 527   | 477   |
| 14                   | 14                        | 266                        | 272   | 277   | 507                                            | 493   | 503   |
| 15                   | 15                        | 256                        | 259   | 266   | 510                                            | 530   | 510   |
| 16                   | 16                        | 263                        | 263   | 264   | 530                                            | 527   | 510   |
| 17                   | 17                        | 266                        | 269   | 272   | 493                                            | 465   | 428   |

Table 7

| Chemical Agents                | Nos. of Aqueous Solutions |     |     |     |     |
|--------------------------------|---------------------------|-----|-----|-----|-----|
|                                | 23                        | 24  | 25  | 26  | 27  |
| Magnesium-boron fluoride (40%) | 0.7                       |     |     | 0.7 |     |
| Aluminum-boron fluoride (30%)  | 0.7                       |     |     | 0.7 |     |
| Zinc-boron fluoride (45%)      |                           | 0.8 | 1.5 | 1.5 | 0.8 |
| Tin-boron fluoride (47%)       |                           | 0.7 |     |     | 0.7 |
| Dihydrated oxalic acid         |                           |     | 0.2 |     | 0.1 |
| Maleic acid                    |                           |     | 0.2 |     | 0.2 |
| Monohydrated citric acid       | 0.5                       | 0.5 |     | 0.2 | 0.2 |
| Tartaric acid                  |                           |     |     | 0.2 |     |
| Tetraoxymethylene              | 3.0                       | 3.0 | 3.0 | 3.0 | 3.0 |
| Polyethylene (softener)        | 2.0                       | 2.0 | 2.0 | 2.0 | 2.0 |

The resultant test samples 23 to 28 were tested their crease resistance and tear strength in the same manner as in Example 1. The test results are given in the following Table 8. As it is obvious from the Table 8, the test samples 23 to 28 have the good and stable crease resistance and tear strength even if the heat treatments are conducted at the different temperatures.

3. The method for imparting crease resistance and soft touch to material selected from cellulosic fibers and textile fabrics and knitted goods containing the cellulosic fibers as claimed in claim 1, wherein the treatment is conducted at a temperature of about 130°C. for 1 to 3 minutes.

4. The method for imparting crease resistance and

Table 8

| Nos. of Test samples | Nos. of Aqueous solutions | Crease Recovery Angle(dry) |       |       | Tear Strength (g) in the direction of the warp, treated |       |       |
|----------------------|---------------------------|----------------------------|-------|-------|---------------------------------------------------------|-------|-------|
|                      |                           | 130°C                      | 140°C | 160°C | 130°C                                                   | 140°C | 160°C |
| 23                   | 23                        | 274                        | 278   | 281   | 542                                                     | 530   | 510   |
| 24                   | 24                        | 280                        | 281   | 284   | 513                                                     | 507   | 495   |
| 25                   | 25                        | 275                        | 277   | 280   | 535                                                     | 523   | 505   |
| 26                   | 26                        | 282                        | 283   | 283   | 508                                                     | 498   | 495   |
| 27                   | 27                        | 284                        | 285   | 287   | 500                                                     | 490   | 490   |
| 28                   | 28                        | 279                        | 280   | 281   | 540                                                     | 505   | 496   |

What I claim is that:

1. A method for imparting crease resistance and soft touch to a material selected from cellulosic fibers, and textile fabrics and knitted goods containing cellulosic fibers comprising treating said material at a temperature of about 120°C to 130°C with 0.1 to 10% tetraoxymethylene in the presence of a catalytic mixture of 0.02 to 10% of a metal-boron fluoride and 0.02 to 10% of an organic carboxylic acid, said percentages being by weight of said material.

2. The method for imparting crease resistance and soft touch to material selected from cellulose fibers, textile fabrics and knitted goods containing the cellulosic fibers as claimed in claim 1, wherein the treatment is conducted at a temperature of about 130°C.

soft touch to material selected from cellulosic fibers and textile fabrics and knitted goods containing the cellulosic fibers as claimed in claim 1, wherein said metal-boron fluoride is selected from a member of the group consisting of magnesium-boron fluoride, aluminum-boron fluoride, zinc-boron fluoride, cadmium-boron fluoride, tin-boron fluoride and lead-boron fluoride, and said organic carboxylic acid is selected from a member of the group consisting of formic acid, oxalic acid, malonic acid, succinic acid, maleic acid, maleic acid anhydride, glycolic acid, lactic acid, malic acid, citric acid and tartaric acid.